

July 24, 1928.

1,678,230

G. A. RICHTER

# PROCESS FOR THE PRODUCTION OF HIGH ALPHA CELLULOSE FIBER

Original Filed April 28, 1925



## UNITED STATES PATENT OFFICE.

GEORGE A. RICHTER, OF BERLIN, NEW HAMPSHIRE, ASSIGNOR TO BROWN COMPANY,  
OF BERLIN, NEW HAMPSHIRE, A CORPORATION OF MAINE.

## PROCESS FOR THE PRODUCTION OF HIGH-ALPHA-CELLULOSE PULP.

Application filed April 23, 1925, Serial No. 26,362. Renewed July 9, 1927.

This invention relates to the utilization of the heat and the recovery of spent sodium digesting constituent from the spent liquor of a plant producing high alpha-cellulose pulp,—that is, pulp containing a high percentage of alpha or resistant cellulose,—where operated simultaneously with a plant producing soda pulp.

High alpha-cellulose pulp may be produced by an alkaline digestion of, for example, unbleached sulphite pulp,—a caustic soda, soda ash, or mixed solution of caustic soda and soda ash being especially adapted for such digestion. The alkaline digestion may take place in digesters at any suitable temperatures and pressures, although I have found it to be more economical and expedient in certain cases to digest the sulphite pulp in open tanks under atmospheric pressure. The alkaline solution reacts with and dissolves the lignin and the less-resistant beta and gamma celluloses contained in the sulphite pulp, and after a sufficient period of digestion yields a pulp product which contains about 94% alpha-cellulose and has a very white color after bleaching. In order to secure a marked economy in the production of high alpha-cellulose pulp, the sodium constituent present in the spent digesting liquor should be recovered, and the available heat content of such liquor utilized.

In companion application Serial No. 26,231, filed April 28, 1925, there has been outlined a process for the recovery of the spent sodium constituent and the utilization of the available heat content of the spent digesting liquor. Such a process, however, requires a special recovery plant, where it is practiced in a plant wherein sulphite pulp only is produced. The object of this invention is to provide a method for practicing the economies set forth in the co-pending application, while combining the recovery of sodium constituent from the spent liquor in an alpha-cellulose plant with the recovery of sodium from the spent black liquor of a soda plant,—thereby obviating the necessity for special recovery apparatus in the alpha-cellulose plant. The manner in which this object is attained, and certain other features of invention revolved in the process, may best be understood from the following description, when taken in connection with the accompanying diagrammatic drawing which

represents what may be termed a "flow sheet."

Before proceeding to the specific features of invention involved herein, the operation of the alpha-cellulose plant (which has been fully described in the companion application) will be briefly reviewed.

Sulphite stock is obtained, as usual, by the digestion of wood chips in a digester under the requisite heat and pressure conditions for the necessary period of time, in a suitable sulphite liquor, as, for example, calcium bisulphite liquor. The digester contents are then blown, and the sulphite stock is successively washed, screened, and thickened by press rolls, to, say, about a 50% consistency. The thickened unbleached sulphite stock thus obtained is delivered to a digesting tank A, communicating by a slow-moving worm conveyor to the bottom portion of a second digesting tank B. The stock is continuously fed into the tank A and is diluted to about a 10% consistency with the required amount of caustic soda or soda ash solution and water, and the stock is fed by the worm conveyor to the tank B, at the same rate at which it is made up in the tank A. The stock is digested with agitation during its passage through the digesting tanks, at from 180° F. to 212° F., under atmospheric pressure, by blowing live steam directly into the stock suspension in the tanks,—the less-resistant beta and gamma celluloses and the ligneous matter contained in the sulphite pulp reacting with and being dissolved by the caustic soda solution, and leaving a pulp containing a high percentage of alpha-cellulose. The agitation provided for during the digestion and the feed of the stock from one tank to the other secures intimate contact between the stock and the cooking liquor, thereby promoting a thorough reaction and resulting in a uniform product. The digestion may be practiced on a batch basis, but obviously a continuous cyclic operation is preferable.

The digested stock, together with the spent digesting liquor associated therewith leaving the top portion of the tank B and now containing a high percentage of alpha-cellulose, is passed through a counter-current washer, wherein the stock is thoroughly washed free from substantially all the spent digesting liquor, and the washed stock is then passed

to the bleachery. The wash water used in the washer assumes practically the same temperature as the hot spent digesting liquor and the hot pulp, as they are passed into the washer. The hot wash water (which for convenience of designation I term the "alpha spent liquor") contains substantially all the sodium constituent in any form, spent or otherwise, associated with the alpha stock as it was passed into the washer. This hot wash water is re-circulated to the digesting tank A, and comprises in volume approximately the volume of water associated with the pulp after digestion, plus the total volume of wash water used in the washer, minus that portion absorbed by the washed alpha pulp as it passes to the bleachery. During this stage of the process, the volume of wash water employed in washing the digested stock is so regulated that the volume of spent alpha liquor obtained from the washer and re-circulated into the tank A is substantially equal to the volume of water and digesting solution employed in making up the initial 10% stock suspension in the tank A. To this recirculated alpha spent liquor is continuously added a sufficient quantity of 50% sulphite pulp, and the amount of concentrated caustic soda or soda ash solution necessary to effectively remove the impurities contained in the sulphite pulp,—thereby again producing a stock suspension of about 10%. The 10% stock suspension formed with the recirculated spent liquor is digested, and the cycle of operations as hereinbefore described in connection with the initial 10% stock suspension, is repeated. The hot spent alpha liquor obtained from the washer at this point in the process contains a higher per cent of dissolved material. This liquor is re-circulated as before, and the process, as described, is continued or repeated until a hot, syrupy spent liquor of about 10° to 15° Baumé results. Such a concentrated spent liquor may profitably be evaporated, and the combustible content thereof burned, to recover the valuable sodium constituent.

When this concentration of spent liquor is reached, the flow of fresh water to the washer is increased. As stated previously, up to this point the volume of spent liquor delivered from the washer has been only sufficient to dilute the incoming unbleached sulphite stock to a 10% consistency, or sufficient to ensure such consistency when the volume of solution containing fresh digesting constituent is taken into account; but there is now an excess of spent liquor. This excess is continuously withdrawn from the spent alpha liquor obtained from the washer and mixed with the black liquor resulting from a soda pulp digestion as it is being passed to the evaporators. The rest of the spent alpha liquor is re-circulated to the alpha digesting tank A. The increase in quantity of wash

water,—that is, the excess passed along with the black liquor to the evaporators,—is so adjusted as to maintain an equilibrium within the system at this particular concentration: that is, the excess spent liquor mixed with the spent soda liquor contains substantially the amount of spent sodium constituent which was formed in the preceding digestion (the term "sodium" or "sodium constituent" as used in this specification and the appended claims, will, of course, be understood to mean sodium in combined form,—that is, in the form of a sodium compound).

It will of course be further understood that the spent black liquor referred to, as indicated on the drawing, results from the digestion of wood chips under the requisite conditions of temperature and pressure, in a digester, in the usual soda digesting liquor, which consists essentially of a solution of caustic soda and a relatively small amount of soda ash and traces of impurities. After the necessary period of digestion, the soda digester contents are blown into the usual blow pit, and the soda pulp is then passed through a counter-current washer similar to the one in which the high alpha-cellulose pulp is washed. The wash water from the counter-current washer contains substantially all the digesting constituent, spent or otherwise, associated with the soda pulp as it is passed into the washer, is black, and of about a 14° Baumé consistency. In certain cases, it may be desirable to return a relatively small portion of this spent black liquor to the digesters for use in a subsequent soda digestion. The large portion of black spent soda liquor, however, is passed into a storage tank, from which it is continually withdrawn to the evaporators. To this black liquor, as has been already indicated, is added the excess spent liquor of from 10° to 15° Baumé, obtained from the alpha spent liquor, so that a mixture of alpha and black liquors of about the same degree Baumé is passed into the evaporators for concentration. The combustible content of the resulting concentrate is burned, preferably in a combined boiler and smelting furnace, in an oxidizing atmosphere, in the usual manner. The smelt from the furnace consists essentially entirely of sodium carbonate, and is run into a dissolving tank containing just enough water to form a concentrated boiling solution of sodium carbonate. The amount of sodium carbonate solution which together with the unspent sodium constituent present in the re-employed alpha spent liquor is necessary for effective digestion of the unbleached sulphite stock fed into the digesting tank A, is continuously withdrawn from the smelt solution, is filtered in the usual manner, and mixed with that portion of the spent alpha liquor which is re-circulated for re-employment in the alpha digesting tanks.

The remainder of the smelt solution is passed into a causticizing tank wherein the sodium carbonate is converted into caustic soda with lime. The precipitated calcium carbonate may then be removed by filtration, and the clear white caustic soda solution obtained may be employed in effecting the next soda pulp digestion. Losses in both the alpha and the soda digestion cycles may be made up by the addition of sufficient soda ash to the smelt solution prior to causticization. With caustic soda more readily available, as in a mill where caustic soda is produced by the electrolysis of salt (NaCl) solution, the losses may be made up by the addition of caustic soda to the white liquor subsequent to causticization as it is passed to the soda digester.

Since sodium carbonate cooking liquor is as effective as caustic soda digesting liquor in the production of high alpha-cellulose fiber, the hereinbefore described process, while possessing all the advantages incident to the co-pending application and eliminating the necessity for special recovery apparatus in an alpha-cellulose fiber plant, also effects an economy in lime equivalent to that which otherwise would be necessary to causticize an amount of soda ash equivalent to the losses experienced in the alpha digesting cycle: that is to say, if the losses in the alpha digestion cycle were added in the form of caustic soda on the alpha side of the drawing, instead of on the soda side of the drawing, more lime would be consumed in the causticization than is consumed by the method described. Of course, the method of recovery of the sodium constituent from the alpha fiber plant when practiced in connection with the recovery of sodium constituent from the soda plant is susceptible of various modifications which are at once apparent to those skilled in the art, and which lie within the spirit of this invention as defined by the appended claims; and, while I have confined myself to the description of what is the preferred method of practicing such recovery in a particular instance, it is not the intention that this description shall have a limiting effect on the invention.

I do not herein claim features generic to application, Serial No. 72,522, filed December 1, 1925, by Milton O. Schur and myself, nor do I herein claim the process disclosed in my applications, Serial No. 26,361, filed April 28, 1925, and Serial No. 28,339, filed May 6, 1925.

What I claim is:

1. A process which comprises digesting predigested pulp in an alkaline liquor containing sodium compounds, re-employing one portion of the spent liquor in another digestion of like pulp and recovering the sodium compounds in the other portion of spent liquor, together with the sodium com-

pounds contained in the spent liquor resulting from the production of pulp from raw cellulosic material.

2. A process which comprises digesting predigested pulp in an alkaline liquor containing sodium compounds, re-employing one portion of the spent liquor in another digestion of like pulp, and mixing the other portion of spent liquor containing substantially the amount of spent sodium formed in a previous digestion with spent liquor containing sodium compounds resulting from a digestion of raw cellulosic material, recovering the sodium constituent of said mixed liquors, using one part of the recovered sodium constituent necessary to effect another digestion of predigested pulp with the re-employed portion of spent liquor, and using the other part in the production of pulp from raw cellulosic material after the addition thereto of sufficient sodium constituent to make up losses suffered in both digesting cycles.

3. A process which comprises digesting unbleached sulphite pulp in an alkaline liquor, re-employing one portion of the hot spent liquor in another digestion of like unbleached sulphite pulp, passing the other portion, together with the spent liquor from a soda pulp digestion, into the recovery system of the soda plant, and recovering the sodium constituent of the mixture.

4. A process which comprises digesting predigested pulp in an alkaline digesting liquor containing sodium compounds, re-employing one portion of the hot spent liquor in another digestion of like pulp, mixing the other portion containing an amount of spent sodium equivalent to that which was formed in a preceding digestion with the spent liquor containing sodium compounds resulting from the digestion of raw cellulosic material, receiving the sodium constituent of the mixture, and adding to said re-employed portion the recovered sodium constituent necessary for another digestion of predigested pulp.

5. A process which comprises digesting predigested pulp in an alkaline digesting liquor containing sodium compounds, re-employing substantially all the spent liquor of one digestion in another digestion after the addition of sufficient alkaline agent thereto to make up losses therein for effective digestion, continuing such re-employment until a predetermined sodium concentration results therein, and thereafter re-employing one portion of the spent liquor in another digestion of like pulp, mixing the other portion containing an amount of sodium equivalent to that which was formed in a previous digestion with liquor containing sodium compounds, resulting from the digestion of raw cellulosic material, recovering the sodium constituent of the mixture, and

adding to said re-employed portion of spent liquor the recovered sodium constituent necessary for another digestion of predigested pulp.

5 6. A process which comprises digesting predigested pulp in an alkaline liquor containing sodium compounds, mixing spent liquor resulting from such digestion with spent liquor resulting from soda digestion 10 of raw cellulosic material, and recovering the sodium constituent of the mixture.

7. A process which comprises digesting predigested pulp in an alkaline liquor containing sodium compounds recovered from 15 the spent liquor resulting from the digestion of raw cellulosic material in the production of soda pulp together with the spent liquor resulting from digestion of predigested pulp with alkaline liquor.

20 8. A process which comprises digesting sulphite pulp under heat in an alkaline liquor containing sodium compounds, mixing a portion of the spent liquor resulting from such digestion with the spent black liquor 25 resulting from soda digestion of raw cellulosic material, recovering the sodium constituent from the mixture, and using part of such recovered sodium constituent in another digestion of sulphite pulp and part for the 30 digestion of raw cellulosic material.

9. A process which comprises digesting predigested pulp under heat in an alkaline liquor containing sodium compounds, re-employing one portion of the hot spent liquor 35 of such digestion in another digestion of predigested pulp, mixing the other portion with the spent black liquor resulting from soda digestion of raw cellulosic material, recovering the sodium constituent of the mixture, 40 and using part of said recovered sodium constituent in the digestion of raw cellulosic material and part in another digestion of predigested pulp together with said re-employed portion of spent liquor.

45 10. A process which comprises digesting predigested pulp under heat in an alkaline

liquor containing sodium compounds, re-employing one portion of the hot spent liquor resulting from digestion in another digestion of predigested pulp, mixing the other portion containing substantially the amount of spent sodium constituent formed in a preceding digestion with the spent black liquor resulting from soda digestion of raw cellulosic material, recovering the sodium constituent of the mixture in the form of sodium compounds suitable for the digestion of predigested pulp, using part of the recovered sodium compounds together with the re-employed portion of spent liquor, in another digestion of predigested pulp, converting the other part into sodium compounds suitable for the digestion of raw cellulosic material, and adding sufficient sodium constituent to said other part to make up sodium constituent losses in both digesting cycles.

11. A continuous cyclic process which comprises continuously feeding and digesting pulp under heat in an alkaline solution of sodium compounds, washing the resulting pulp and the entrained products of the reaction, circulating a part of the hot wash water back for further digestion of pulp, mixing the other part with the black spent liquor resulting from a soda digestion, evaporating said mixed spent liquor, burning the organic content and smelting the inorganic content thereof in an oxidizing atmosphere so as to give a smelt consisting essentially of sodium carbonate, recovering the molten smelt in water, mixing one portion of the resulting hot liquor with the recirculated wash water, causticizing the remaining portion with lime, filtering it, re-employing said filtered white liquor in a subsequent soda pulp digestion, and making up losses in both digesting cycles by the addition of sodium digesting agent to said filtered liquor.

In testimony whereof I have affixed my signature.

GEORGE A. RICHTER.